

A. J. ISRAEL.  
PROCESS OF LINING METAL PIPES AND THE LIKE.  
APPLICATION FILED DEC. 10, 1919.  
**1,368,632.**

Patented Feb. 15, 1921.



Inventor:  
Aaron Jacob Israel  
By Lawrence Daupner  
Attorney.

# UNITED STATES PATENT OFFICE.

AARON JACOB ISRAEL, OF JOHANNESBURG, TRANSVAAL, SOUTH AFRICA.

## PROCESS OF LINING METAL PIPES AND THE LIKE.

1,368,632.

Specification of Letters Patent. Patented Feb. 15, 1921.

Application filed December 10, 1919. Serial No. 343,959.

To all whom it may concern:

Be it known that I, AARON JACOB ISRAEL, a British subject, residing at "Moresby," 140 St. John's road, Houghton Estate, Johannesburg, Transvaal Province of the Union of South Africa, have invented certain new and useful Improvements in Processes of Lining Metal Pipes and the like, of which the following is a specification.

10 The present invention has reference to the lining of metal pipes for the purpose of protecting them against corrosion or wear by acid water or other corrosive or abrasive liquid. The invention is also applicable to

15 the lining of metal pipes which in use have become worn or pitted, for the purpose of rendering them again serviceable.

According to the present invention a lining of cementitious material is formed centrifugally within the metal pipe. Various cementitious materials may be used and satisfactory results have been attained with a concrete formed of Portland cement and sand, the consistency of the admixture being

25 such as to readily flow.

In carrying out the process the metal pipe is mounted in suitable apparatus for revolving it preferably at speed which can be varied. The ends of the metal pipe are partially closed by means providing an inward flange, and the cementitious material in admixture with water, is introduced into the metal pipe in such quantity, having regard to the length of the pipe, as to form, when set, a liner of the required thickness. The pipe is revolved at such a speed as to spread the cement evenly along and around the interior of the pipe. Thereafter the speed of rotation is increased so as to rapidly eliminate the surplus water and to cause the cement to settle. Such surplus water may be withdrawn from the opening of the pipe by appropriate method or means hereinafter described and rotation of the pipe is continued until the cement is sufficiently set to enable the pipe to be handled. In practice it has been found that the foregoing operations can be carried out in a period of approximately ten minutes. The pipe is then withdrawn from the apparatus in which it is rotated and laid aside to permit the setting of the cement to be completed.

50

The accompanying drawings show apparatus suitable for carrying the invention into effect.

Figure I is a perspective view partly in

section of a device for attachment to the end of the pipe for partially closing the same.

Fig. II is a partly sectioned side elevation of a modified attachment.

60

Fig. III is a side elevation of a pipe rotating machine.

Referring to Fig. I, 1 indicates the metal pipe which is to be lined. For the purpose of partially closing the end of the same a halved clamp 2 is secured to the pipe at a little distance from each end. A disk 3 is positioned against the end of the pipe, and is held in place by bolts 4 passing through the clamp 2. The disk 3 is formed with a central aperture 6 equal in diameter to the internal diameter of the liner to be formed. In the wall of said aperture 6 is formed an annular groove 7 in which is seated a split ring 8 and a recess 9 is formed to give access to the ends of the ring 8 for the purpose of removing said ring. In employing this device one is bolted to each end of the metal pipe, as described, with the split ring 8 in place. After the pipe has been sufficiently revolved to settle the cement, and bring the superfluous water to the interior, the rotation is stopped and the ring 8 removed by inserting a suitable tool in the recess 9 and forcing in the free ends of said ring. Removal of the ring 8 permits the superfluous water to escape, whereafter the rotation is continued until the cement is sufficiently set to permit the metal pipe to be removed from the rotating machine. The end closing device 2, 3 may thereafter be removed from the pipe and utilized on another pipe which is about to be lined. In the case of a pipe having a flange at its end the disk 2 is secured directly to the said flange.

75

80

85

90

95

The end closing device shown in Fig. II is designed to be used in conjunction with the regular screw socket 10, by which pipes having threaded ends are connected. The device comprises a cylindrical portion 11 externally threaded to screw in such socket and up to the end of the pipe 1. At its outer end is formed a head 12 which is polygonal or otherwise formed for engagement of a spanner or other implement for turning it. 100 In the said head is formed the groove 7 in which is seated the split ring 8 described in connection with Fig. I. The internal diameter of the part 11 and of the aperture 6 is made equal to the internal diameter of the liner desired and the ring 8 is, as before, of somewhat smaller internal diameter.

110

While it is obvious that many different kinds of apparatus may be employed for rotating the pipe, that shown in Fig. III has been specially designed for the purpose and 5 has proved satisfactory. It consists of a bed 13 on which are mounted a fixed head stock 14 and a tail stock 15 traversable along the bed by suitable means such as the pinion 16 engaging the rack 17. The head stock 10 and tail stock are each provided with a rotatable hollow mandrel 18 and each such mandrel is provided, preferably at its outer end, with a hollow chuck 19. Said hollow chucks are arranged to grip the metal pipes 15 and are preferably self centering chucks, as shown. The mandrel 18 of the head stock is provided with means for rotating it, such as the belt pulley 20.

In using the machine the pipe is passed 20 through the two hollow chucks so as to project to a reasonable extent beyond the end of each, and the chucks are then tightened up after the tail stock has been traversed to a suitable position along the bed 25 13. The hollow mandrel 18 of the head stock, is then rotated, so rotating the pipe 1 and with it the mandrel of the tail stock.

I claim—

1. The process of lining metal pipes with cementitious material, which consists in 30 partly filling the pipe with a mixture of cementitious material and water of such consistency as to readily flow; preliminarily rotating the pipe at relatively low speed to spread the cementitious material around 35 and along the interior of the pipe; and then rotating the pipe at relatively high speed to remove the surplus water from the cementitious material and set the lining.

2. The process of lining metal pipes with 40 cementitious material, which consists in partially closing the end of the pipe to be lined; partly filling the pipe with a mixture of cementitious material and water of such consistency as to readily flow; preliminarily rotating the pipe at relatively low speed to spread the cementitious material around 45 and along the interior of the pipe; and then rotating the pipe at relatively high speed to remove the surplus water from the cementitious material and set the lining.

In testimony whereof I affix my signature.

AARON JACOB ISRAEL.